

## UNITED STATES PATENT OFFICE

GEORGE HOLLAND ELLIS, OF SPONDON, NEAR DERBY, ENGLAND, ASSIGNOR TO CELANESE CORPORATION OF AMERICA, A CORPORATION OF DELAWARE

## TREATMENT OF MATERIALS MADE OF OR CONTAINING CELLULOSE DERIVATIVES

No Drawing. Application filed March 25, 1927, Serial No. 178,505, and in Great Britain October 30, 1926.

This invention relates to the mordanting of yarns or threads, or woven, knitted or other textile fabrics, films or other products made of or containing cellulose acetate or other organic acid esters of cellulose, for example cellulose formate, propionate or butyrate, or made of or containing cellulose ethers, such as methyl, ethyl or benzyl cellulose or the corresponding condensation products of cellulose and glycols or other polyhydric alcohols, all of which are hereinafter referred to as organic substitution derivatives of cellulose.

In dyeing cellulose acetate materials by first mordanting and then dyeing, it has previously been proposed to apply the metallic mordants in the form of thiocyanates.

It has now been found that the absorption of the mordant by the cellulose acetate materials is largely influenced by the concentration of the thiocyanate grouping present in the mordanting liquor quite apart from the concentration of the metallic radicle itself. Thus, by increasing the concentration of the thiocyanate radicle compared with that of the metallic radicle, it has been found possible to effect a higher degree of absorption of the metallic radicle than with a mordanting liquor containing the same concentration of metallic radicle together with the chemically equivalent concentration of thiocyanate radicle, or alternatively to effect an equivalent degree of mordanting to that obtainable with molecular proportions of metal and thiocyanate whilst using a considerably lower concentration of the metallic radicle.

This mordanting process, i. e. using higher than molecular concentrations of thiocyanate, is further applicable to the mordanting of materials made of or containing any other of the aforesaid organic substitution derivatives of cellulose.

Accordingly the present invention comprises mordanting materials made of or containing cellulose acetate or other of the aforesaid organic substitution derivatives of cellulose with solutions or pastes containing the thiocyanate radicle in a concentration in excess of that which is chemically equivalent

to the mordant metal radicle present in the solution or paste.

The increase in the thiocyanate concentration may for example be effected by addition to the thiocyanate of the mordant metal or metals of a thiocyanate of a base not showing mordant properties, for instance ammonium thiocyanate or sodium or potassium thiocyanate, or alternatively such a thiocyanate may be added to a salt of a mordant metal in excess of the chemically equivalent quantity.

The improved absorption of the mordants enables the operation of mordanting to be carried out more expeditiously, or more conveniently in bulk practice, and effective mordanting may for example be achieved by continuous means, the material being merely passed through the mordanting liquor, the superfluous liquor preferably squeezed out, and the materials allowed to lie until the maximum amount of mordanting has taken place.

In addition to an intensification of mordanting resulting in advantages in time, temperature, concentration and manipulative factors, the method according to the present invention is also advantageous in that it diminishes the risk of obtaining a surface deposit of the mordant with consequent tendency of the dyeing or coloring to rub off or to be less lustrous.

In carrying out the invention so as to mordant the whole of a fabric, the fabric may be brought into a liquor containing a thiocyanate of a metallic radicle desired for or capable of yielding results in mordanting, such for example as iron, aluminum, chromium and the like (or mixtures of such) and a thiocyanate of a non-mordanting metal base, such as ammonium, sodium or potassium thiocyanate.

The amount of mordant required will usually be governed by the depth of shade ultimately desired, and the concentration, temperature and time of treatment may be varied accordingly.

The following examples are given by way of illustration, it being understood that they are in no way limitative.

*Example 1*

To mordant 100 lbs. of cellulose acetate woven fabric with iron. The cellulose acetate material is treated in any suitable manner for about 1 hour at about 75° C. in a bath (approximately 30:1 on the goods) made up with liquor so as to contain 54 grams of ferric chloride (0.33 gram molecules) and 152 grams of ammonium thiocyanate (2 gram molecules) per litre. The material is then removed and washed off first in cold and then in warm water until there is a change in shade from a deep red to a golden yellow color. The hydrolysis of the thiocyanate of iron may conveniently be completed by treatment in a separate bath containing 5 grams of sodium carbonate per litre at 30-35° C. for 5-10 minutes. After rinsing, the goods are ready for the dyeing operation.

*Example 2*

A similar mordanting result to that obtained according to the process of Example 1 may be achieved alternatively in a manner especially suitable to bulk production. The fabric is passed continuously by means of any suitable machine through a liquor containing ferric chloride and ammonium thiocyanate in similar concentrations to those used in the foregoing example. The fabric, after passage through the liquor, being squeezed between rollers adjusted so that the goods retain about their own weight of liquor. The temperature may conveniently be adjusted to about 50° C. After squeezing the goods are allowed to lie for about 12 hours, conveniently overnight. They are then subjected to washing and/or sodium carbonate treatment for hydrolysis of the thiocyanate of iron as described in Example 1. The goods may then be dyed as desired, for example a full black shade may be produced by treatment at about 75° C. in a bath containing 10% haematin crystals on the weight of the goods.

*Example 3*

To mordant with chrome 100 lbs. of cellulose acetate yarn in the form of hanks. The goods are treated for 1 hour at about 75° C. in a bath having a ratio to the goods of approximately 30:1 and containing 53 grams of chromium chloride (0.33 gram molecules) and 114 grams of ammonium thiocyanate (1.5 gram molecules) per litre. After this treatment the cellulose acetate material is washed off at 30° C. for 5-10 minutes in a solution of soda ash (5° Tw.). Subsequently the material is rinsed in soft water. The yarn may then be dyed as desired, for instance if dyed with 2% alizarine on the weight of the goods at 75° C. a deep maroon color is obtained.

*Example 4*

To mordant with aluminium 100 lbs. of cellulose acetate knitted fabric. The fabric is treated for 1 hour at 75° C. in bath of approximately 30:1 ratio to the goods and containing 107 grams of aluminium chloride (0.8 gram molecules) and 274 grams of ammonium thiocyanate (3.6 gram molecules) per litre. The material is then washed off at 30° C. for 5-10 minutes in a solution of soda ash (5° Tw.). The material may subsequently be rinsed in soft water and dyed as desired, for instance if dyed with 2% alizarine on the weight of the goods at 75° C. a bright red is produced.

The process is applicable, in addition to the mordanting and dyeing of the whole of a fabric or other material, to the local application of mordants and mordant dyestuffs for example by printing or stencilling by methods known in the art.

The process of the present invention may be applied to goods composed wholly of cellulose acetate or other of the aforesaid organic substitution derivatives of cellulose, or to mixed goods containing for example, in addition to one or more of the aforesaid organic substitution derivatives of cellulose, wool, cotton, natural silk, artificial silk of the cellulose type etc.

What I claim and desire to secure by Letters Patent is:—

1. A process of mordanting materials comprising organic substitution derivatives of cellulose, which comprises applying the metallic mordants thereto in the form of thiocyanates, the concentration of thiocyanate radicle present being in excess of that chemically equivalent to the mordant metal radicle.

2. A process of mordanting materials comprising cellulose acetate which comprises treating the materials in a solution of the thiocyanate of the mordant metal containing the thiocyanate radicle in a concentration in excess of that chemically equivalent to the mordant metal radicle.

In testimony whereof I have hereunto subscribed my name.

GEORGE HOLLAND ELLIS.